

No. 858,622.

PATENTED JULY 2, 1907.

A. J. PETERSSON,  
METHOD OF CARRYING OUT METALLURGICAL REDUCTION AND MELTING  
PROCESSES.  
APPLICATION FILED OCT. 30, 1906.

FIG: 1.



FIG: 2.



Witnesses.

*P. Dommers*  
*Jesse K. Lutton*

Inventor.

*Albert Johan Petersson*  
by  
*Henry Otho*  
att.

# UNITED STATES PATENT OFFICE.

ALBERT JOHAN PETERSSON, OF ALBY, SWEDEN.

## METHOD OF CARRYING OUT METALLURGICAL REDUCTION AND MELTING PROCESSES.

No. 858,622.

Specification of Letters Patent.

Patented July 2, 1907.

Application filed October 30, 1906. Serial No. 341,343.

To all whom it may concern:

Be it known that I, ALBERT JOHAN PETERSSON, a subject of the King of Sweden, and resident of Alby, Sweden, have invented certain new and useful Improvements in Methods of Carrying Out Metallurgical Reduction and Melting Processes; and I do hereby declare the following to be a full, clear, and exact description of the invention, such as will enable others skilled in the art to which it appertains to make and use the same; reference being had to the accompanying drawings, and to letters or figures of reference marked thereon, which form a part of this specification.

This invention relates to a method of carrying out metallurgical reduction- and melting-processes by means of electricity, the said method rendering it possible to obtain a higher efficiency from the electric current than theretofore. The method may especially be used for such reduction processes where as a reduction means carbon or carbonic acid is used.

20 The chief object of the invention is to utilize in an economical manner the excess of carbonic acid formed in the reduction process for preliminary heating the charge. The invention, however, is not limited thereto, the general object of the same being to obtain an effective preliminary heating of the charge by burning combustible gases in the same, whether the said gases are formed during the process or are supplied from without.

30 The invention consists, principally, in charging successively into the furnace anthracite coal, or the like, hereinafter referred to as carbon, and the ore, or the like, to be reduced in such a manner that they continually form separate columns, and burning combustible gases in the column or columns of ore, or the like, for preliminary heating the same before it comes into the reduction zone of the furnace. The said method is a simple and effective manner of utilizing the excess of carbonic acid formed in the reduction process, it being only necessary to arrange the furnace so that the said

40 gas flows off through the column of ore, or the like, and to introduce into the said column a suitable quantity of air for burning the carbonic acid into carbonic acid.

In the usual processes in which the ore and the carbon are charged into the electric furnace mixed with each other it has not been possible to carry out such a combustion of the carbonic acid in the charge, the carbonic acid causing the combustion of a part of the carbon of the charge as well as a part of the electrodes so that it would have been impossible to determine correctly the proportions between the carbon and the ore of the charge as is necessary for carrying out the process continuously and economically. In the processes above mentioned it has been necessary to burn the carbonic acid in special roasting-and-combustion-furnaces, which process, obviously, is not economical, in as much as the ore will lose a good deal of its heat be-

fore reaching the reduction zone of the electric furnace. It has also been proposed to burn combustible gases in such electric furnaces where the ore and the carbon are charged in separate layers but in said furnaces the combustion has taken place in the layer of carbon and while it is important to obtain the highest temperature possible in the charge of ore or the like heated by the electric current by heating the surrounding layers of carbon to the highest temperature possible no consideration has been taken to the consumption of carbon and electrodes.

In the present invention the combustion of the gases can take place in close proximity to the reduction zone so that the ore, or the like, will be preliminarily heated thereby immediately before it comes into the said zone, and simultaneously the charge of carbon as well as the electrodes may be prevented from being consumed in any essential degree by the said burning of gases, in as much as the electrode or electrodes may be arranged in the column or columns of carbon and the latter may be kept so compact that neither the carbonic acid nor the air introduced into the column of ore, or the like, will in any essential degree take their way therethrough. The combustion of gas may be so directed that the gas and air partaking in the combustion flow from the column or columns of carbon toward the outlets for the products of combustion.

The invention will be more particularly described herebelow with reference to the accompanying drawing showing substantially diagrammatically an electric furnace for carrying out the process.

Figure 1 is a side-elevation partly in section and Fig. 2 is a plan-view partly in section on line II-II of Fig. 1.

Referring to the drawing, the furnace shown has three shafts 1, 2 and 3 of which the shafts 1 and 3 are adapted to be charged with ore, or the like, while the shaft 2 is adapted to be charged with carbon, coke, anthracite, char-coal, or the like. The upper part of the inner shaft walls may be made hollow, as shown, for the purpose of reducing their weight, such reduction being desirable as the walls are not supported at their base. At the bottom the three shafts form a single reduction- and melting-zone forming a part of a circulation system 100 which consists of regenerators 4 and 5 provided on each side of the reduction zone; a pipe 6 between the outer ends of the regenerators and a fan 61 or other circulation device inserted in the pipe, whereby the gases contained in the circulation system may be brought to circulate 105 through the reduction zone in the one direction or the other. When the process has been started the said gases consist chiefly of carbonic acid which will be heated to a high temperature when passing through the column of carbon and thereupon when passing through the column of ore next to the column of carbon, counted in the direction of flow, be converted into carbonic acid

which when passing through the column of carbon will be reduced to carbonic oxide. In as much as in said reduction an excess of gas will be formed corresponding to one molecule of carbonic oxide for each reduced 5 atom of oxygen it will be necessary to lead off when the process is going on a certain quantity of the gas from the system. According to the present invention this is carried out in such manner that the excess of gas is allowed to rise through the shafts 1 and 3 containing 10 ores, or the like, while simultaneously air is introduced into the said shafts, the said air causing a combustion of the gases flowing off in the columns of ore above the reduction zone. For such purpose the furnace illustrated in the drawing is provided with channels 7, 8 and 15 9, 10 in the side-walls of the shafts 1 and 3 respectively, the said channels communicating by means of a number of openings 14 and 15 respectively with the interior of the shafts and being at their outer ends in communication with a pipe 16 containing a fan, or the like, 17 for 20 forcing the air into the shafts. In order to prevent the said air from flowing down to the gas partaking in the circulation, whereby it would cause a useless combustion of the carbon of the charge, the combustion of the excess of gas is suitably so directed that it takes place 25 alternately in the one shaft and the other. For said purpose valves 18, 19, 20 and 21 are inserted in the branch-pipes 161, 162, 163, and 164 between the pipe 16 and the channels 7, 8, 9 and 10, and in the outlet-pipes 22 and 23 are inserted valves 24 and 25 respectively. 30 The positions of the said valves should be changed, when the direction of circulation is reversed, in such a manner that the valves corresponding to the shaft that is after the column of carbon counted in the direction of flow are closed. The flow of gas which enters into the 35 reduction zone from one of the regenerators will hereby be divided so that the excess of gas flows up through the overlying layer of ore and is there mixed with the air forced in, the said air effecting a combustion of the gas flowing off while heating the ore.

40 Instead of forcing the air into the furnace for burning the excess of gas in some cases I draw out the said excess

and simultaneously draw in air through the column of ore, or the like, the said air thereby effecting a burning of the gas before leaving the furnace. This is especially suitable in such cases where the carbon works a direct 45 reduction, for instance in the production of silicious iron by melting scrap iron and silicic acid by means of electrically heated carbon, the circulation of gas being in such case dispensable.

By the above described combustion of gases the consumption of electric current can obviously be considerably reduced, in as much as the electric current need not be used for heating the charge of ore to the reduction temperature.

Having now particularly described my invention, 55 what I claim as new and desire to secure by Letters Patent is:

1. The method of reducing and melting ores and the like in an electric furnace which consists in introducing the ore to be treated and the carbon used for the reduction in the furnace in such a manner that they continuously form separate upright columns in close contact with each other, leading an electric current through the column of carbon for heating the same to a temperature sufficient for reducing the ore, and burning the combustible gases 60 formed during the reduction process in the column of ore for preliminary heating the same, substantially as and for the purpose set forth.

2. The method of reducing and melting ores and the like in an electric furnace which consists in introducing 70 the ore to be treated and carbon used for the reduction in the furnace in such a manner that they continuously form separate upright columns in close contact with each other, leading an electric current through the column of carbon for heating the same to a temperature sufficient for reducing the ore, circulating reducing gases from the 75 column of carbon through the column of ore and then back again to said column of carbon, and burning the excess of said reducing gases in the column of ore for preliminary heating the same, substantially as and for the purpose set forth.

In testimony that I claim the foregoing as my invention, I have signed my name in presence of two subscribing witnesses.

ALBERT JOHAN PETERSSON.

Witnesses:

CARL FRIBERG,  
EWALD DELMAR.